

March 31, 1925.

1,531,530

C. O. WALPER

PROCESS OF PLASTERING

Filed July 20, 1922



Inventor

Curry Ora Walper,

By

Brink & Brink

Attorneys

Patented Mar. 31, 1925.

1,531,530

# UNITED STATES PATENT OFFICE.

CURRY ORA WALPER, OF DETROIT, MICHIGAN, ASSIGNOR, BY DIRECT AND MESNE ASSIGNMENTS, TO STANDARD PLASTERING SYSTEM, OF DETROIT, MICHIGAN, A CORPORATION OF MICHIGAN.

## PROCESS OF PLASTERING.

Application filed July 20, 1922. Serial No. 576,261.

To all whom it may concern:

Be it known that I, CURRY ORA WALPER, a citizen of the United States of America, residing at Detroit, in the county of Wayne 5 and State of Michigan, have invented certain new and useful Improvements in Processes of Plastering, of which the following is a specification.

This invention relates to a system of plastering particularly applicable in providing a finishing coat for a wall board surface.

The primary object of my invention is to provide a finishing coat adapted for use with wall boards having a surface coating of 15 paper or other porous material.

A still further object of the invention is to provide a finishing coating which may be rapidly applied to a porous surface to provide a smooth and uniform finish in a single 20 continuous operation.

The increasing cost of lathing and of labor has led to the provision of many forms of wall boards adapted to be nailed directly to studs and joists without the use of wood or 25 metal lathing. Such boards are commonly made of various forms of paper pulp or of gypsum plaster having a paper surface. In some cases the composition boards consist of 30 various layers of paper, plaster, and other material.

In order to conceal the joint at the meeting edges of such boards various forms of crack fillers have been used, these filling compositions usually consisting of some quick 35 setting mixture of gypsum containing glue or wood flour or other inert materials. However the shrinking and warping of the material of the wall boards due to variations in moisture in the air or in the walls is usually 40 sufficient to cause cracks to form at the meeting edges and other strains such as those due to hammering or strains caused by drying of the studs and joists will also act to produce cracking. It has therefore been deemed necessary to apply upon the surface of such plaster boards a rough coat of plaster, in many cases as thick as the wall board itself, and upon this rough coat a finishing or putty 45 coat. This putty coat commonly consists of lime with a little gypsum added and while the percentage of gypsum may be made as high as fifteen per cent, the tendency on the part of workmen is to use less than this 50 quantity, since in the ordinary manner of

preparation of such mixture a larger quantity of gypsum usually causes difficulty in the application of the coat to the wall surface.

Gypsum ordinarily sets more rapidly than is convenient for the application of a surface coat if it is used in a percentage producing the best results in the ordinary finished wall and the tendency is therefore to reduce the amount to avoid the preparation of numerous small batches of material. By 60 increasing the percentage of lime, a larger amount of wet putty coat may be prepared at one time without danger of injurious setting before it can be applied to the rough coat. This ordinary putty coat is not satisfactory as a surface finish for paper coated 65 plaster boards.

The lime requires a certain amount of moisture during its hardening process to facilitate the rapid absorption of carbon dioxide and to prevent undue shrinkage of the surface during setting. This moisture is usually supplied by water absorbed by the rough coat to which the finishing coat is 70 usually applied.

In the case of plaster boards having a paper surface there is not enough moisture absorbed and retained to cause a proper setting of the lime and it has been found that the ordinary putty coat cannot be used satisfactorily directly upon the surface of the 75 plaster boards as a single unitary finishing coat.

The accompanying drawing indicates in transverse section a wall of plaster board 80 coated in accordance with this invention.

The composition of the primary coating of the present invention consists of a mixture of gypsum fifty per cent to seventy-five per cent, lime fifteen per cent to forty per cent and sand, where sand is used, ten per cent, though the mixture may be used free from sand. The preferred mixture consists of gypsum sixty per cent, lime thirty per cent and sand ten per cent. If the gypsum is as high as seventy-five per cent, the lime may be fifteen per cent and the sand ten per cent. To this mixture of lime, gypsum and sand or lime and gypsum is added a sufficient quantity of water to produce a plastic composition of a consistency adapting it for ready application to the surface of the boards. The quantity of water will vary with 100 105

the degree of porosity of the surface of the boards, a very porous board requiring a mixture containing a greater quantity of water than would be required by a board having a surface only slightly absorbent.

6 A composition having this high percentage of gypsum will cling very tenaciously to a paper or other porous surface and while it is somewhat brittle, it has great elasticity,

- 10 permitting considerable bending without cracking. A sufficient amount of commercial retarder will be used in the preparation of the mixture to prevent too rapid setting of the composition. For best results, the paper 15 surface should be sufficiently porous to absorb a considerable amount of water but should not have enough suction to dry out the plastic mixture to an extent preventing proper setting and hardening of the composition.

15 It is to be observed that whereas in the previous composition used for the ordinary putty coat a small percentage of gypsum is used with a large percentage of lime, the 20 purpose of the gypsum being to produce a rapid setting of the mixture sufficient to prevent injurious shrinking, but the mixture depending for its ultimate hardness upon the conversion of the colloidal hydroxide of 25 calcium into calcium carbonate by the absorption of carbon dioxide from the atmosphere, in the present instance the primary coating depends for its hardness upon the high percentage of gypsum present and upon 30 the sand when the sand is used, the lime together with the retarder being used only for the purpose of producing the smooth flowing mixture capable of being applied as a thin coating upon the surface of the boards.

- 35 40 After the workman has applied a thin coating of this composition having a high percentage of gypsum to the surface of the paper coated boards or to any other suitable porous surface, there will be a certain absorption of moisture which will occur very soon after the application of the coating and if the amount of retarder has been properly regulated the mixture will begin to set very soon after the workman has completed 45 the necessary smoothing of the primary coat. With wall boards of the ordinary type coated with paper a layer three-sixteenths of an inch in thickness has been found to be sufficient.

- 50 55 As soon as the workman has covered the space readily reached from his scaffolding, the material first applied will have set sufficiently to receive the finishing coat. The primary coat should still be wet but even 60 in this condition the gypsum composition will have a considerable suction and will be well adapted to receive the finishing coat.

55 The finishing coat will preferably not contain as high a percentage of gypsum as is 65 contained in the primary coat, since with a

high percentage of gypsum it is difficult to obtain a surface as smooth as is usually desired. By increasing the percentage of lime, a composition which will work much more smoothly is obtained. The preferred percentage of this finishing coat will be lime 70 sixty per cent and gypsum forty per cent, the sand being omitted. A certain amount of commercial retarder will be used to prevent too rapid setting of the gypsum.

75 This finishing coating will be applied smoothly, in a very thin layer, upon the surface of the primary coating which will be set sufficiently to be rigid under the pressure of the plasterer's tools, though it will still be 80 wet with the moisture it contained when it was applied. The plasterer will quickly apply this thin surface coating over the primary coating ready to receive it and by the time he has completed the spreading of the 85 finishing coat, the portion first applied will have lost sufficient moisture by the suction of the primary coating so that it will be ready for the final rubbing in with the 90 finishing tool.

90 It will be seen that by this system the complete finishing coating may be applied to a paper wall board surface or to any other suitable porous surface in what is practically a single operation, with a single 95 setting of the scaffolding. By the use of the compositions described, only a small quantity of material will be required as compared with the ordinary plastered surface and the resulting finish will be smooth and 100 hard.

105 By this system there is provided a primary coating which will adhere tenaciously to a paper surface and which will have great elasticity, and a finishing surface coating which will adhere to the primary coating 110 while having good working qualities enabling a workman to produce a hard smooth and satisfactory surface with a minimum expenditure of labor and time.

110 The system is economical in that it permits the production of a finished surface coating upon a wall board foundation with a small quantity of material rapidly applied without the necessity of waiting for the drying of a rough coat as in ordinary plastering.

115 Lime in the primary coat not only makes it work more smoothly, but also checks the corrosive action of the gypsum on the metal reinforcements used in covering the meeting edges of the boards and the fastening means as described in my co-pending application, Serial No. 576,969.

120 125 The primary coating containing a high percentage of gypsum will adhere to the paper coating of a wall board even when it has been sized to limit the absorption of water by the board. The addition of sand or scoria lengthens the time of setting but 130 does not prevent this adhesion.

However where the percentage of lime is high in proportion to the gypsum, the coating will not cling to the paper when the composition has become dry but may readily be detached. The lime appears to prevent proper adhesion.

The primary coating containing gypsum in high percentages has the peculiar quality of having great suction even while still wet, after it has acquired its set. This feature makes possible the immediate use of the finishing coating with excellent results. In the preparation of this finishing coat, to secure the proper consistency for easy mixing and to slake the lime, a considerable quantity of water is used, which results in a thin mixture. This cannot be properly finished until some of the water is removed. The suction of the wet primary coating is sufficient to remove enough water to bring the finishing coating to a consistency enabling the workman to apply the final troweling with ease.

I claim:—

1. A process of plastering which consists in applying to a porous surface an adhesive quick setting plastic gypsum composition as a primary coating and after the primary

coating has taken its setting but before it has become dry applying to the surface 30 therof a finishing coating of a comparatively slow setting plastic composition containing gypsum.

2. A process of plastering which consists in applying to a porous surface a plastic 35 composition containing gypsum in excess of fifty per cent as a primary coating and after the primary coating has taken its set but before it has become dry applying the finishing coating thereto consisting of a plastic 40 composition containing less than fifty per cent of gypsum.

3. A process of plastering which consists in applying to a porous surface a plastic composition containing lime and gypsum 45 with the gypsum in excess and after the composition has set but before it is dry applying a finishing coating containing lime and gypsum with the lime in excess.

In testimony whereof I affix my signature 50 in presence of two witnesses.

CURRY ORA WALPER.

Witnesses:

ARTHUR MINNICK,  
GEFA L. TERNA.